

## UNITED STATES PATENT OFFICE

2,104,890

PROCESS OF SEPARATING FROM PIG-IRON  
THE VANADIUM CONTAINED THEREIN

Nicolaus Wark, Soureth-Heerlen, Netherlands

No Drawing. Application December 5, 1933, Serial No. 701,081. In Germany December 14, 1932

2 Claims. (Cl. 75—52)

A great part of the ores to be treated in the blast-furnace contains admixtures of vanadium which in practice are again completely present in the pig-iron obtained from the furnace. Thus, for instance, the pig-iron obtained from limonite (minette), contains from 0.10 to 0.25% of vanadium, depending upon the degree of breaking up the ores and other conditions of operation, while pig-iron produced from northern ores by blast-furnaces has a content of vanadium amounting to as much as 1%.

My invention has for its object to devise a process which permits separating from the pig-iron the greatest part of the vanadium contained therein by way of the slag, so that the latter may be further worked economically by the known process into ferro vanadium or other vanadium compounds.

My invention is based on the fact that the course of chemical reactions in metal baths depends to a very large extent upon the thermal, physical and chemical properties of their slags and that certain reactions can be carried out at all only underneath quite definite slags. In case the product obtained by reaction is not afforded the possibility of being taken up and bound by a strongly reacting, very liquid and properly composed slag in its state of unstable equilibrium, it will be exposed to the danger of being carried back into the bath under the influence of other components.

The vanadium contained in the pig-iron, by reason of its great affinity for oxygen due to its position in the periodic system, is strongly subject to oxidation into vanadic acid. This known process could heretofore not be fully utilized for the separation of the vanadium from pig-iron because the other conditions connected with the binding of the vanadic acid have heretofore been left entirely out of consideration. When treating pig-iron containing vanadium by the open-hearth process, first vanadic acid ( $V_2O_5$ ) will be formed, however, almost simultaneously therewith also the silicon contained in the pig-iron will undergo combustion to form silicon dioxide ( $SiO_2$ ). If the slag is inadequately prepared, for instance if said slag is not very liquid and thus incapable of bringing about reaction with all such acid compounds, that is, not sufficiently and effectively basic, the bases present in the slag, such as calcium oxide ( $CaO$ ), manganous oxide ( $MnO$ ) and others by reason of their great affinity for silicic acid will be bound quickly by the latter, so that the vanadic acid in uncombined and unstable condition is reduced by the silicon

in the metal-bath and the vanadium carried back into the pig-iron bath with combustion of the silicon into silicon dioxide ( $SiO_2$ ). Such unprepared slag, therefore, can contain only small quantities of vanadium in combined condition and for this reason is unsuitable for recovering the vanadium from the iron.

According to my invention, on the basis of the above, a strongly basic, well reacting and very liquid slag, for instance a slag having bases which among other compounds contain sodium or potassium compounds, is added to the pig-iron that contains vanadium, preferably before oxidation of the vanadium into vanadic acid commences. This slag in its liquid condition and its strongly basic condition will be capable of practically fully binding the resulting vanadic acid. This vanadic acid is drawn off after complete oxidation of the vanadium and the open-hearth or other refining treatment thereupon is continued underneath a new normal slag. In this manner a fresh slag is obtained which owing to its high content of vanadium permits of economical commercial separation of this metal from the iron. As bases, besides sodium oxide ( $Na_2O$ ) and potassium oxide ( $K_2O$ ), also other substances having a similar effect may be used directly, such as for instance manganous oxide ( $MnO$ ). In order to avoid formation of unnecessarily large quantities of slag having a relatively small content of vanadium—which is due to the fact that the combustion of the silicon takes place practically simultaneously with the combustion of the vanadium—and in order to prevent any vanadium which has already entered into the slag from being carried back into the bath, it is of advantage to first subject the pig-iron to a preliminary open-hearth treatment in order to oxidize the silicon therein underneath a slag rich in silicic acid and to bind the thus formed silicic acid either by lime or metallic bases and draw off the compounds so formed. A vanadium recovery treatment is now carried out underneath the aforementioned basic and very liquid slag after removal of the initial acid slag which contains practically all the silicon. If a pig-iron low in silicon is available as initial material due to properly carrying through the blast-furnace process, the silicon treatment can be dispensed with and the charge may then with advantage be treated directly to separate the vanadium. The composition of the pig-iron is further of importance in so far as a greater content of manganese in the iron during the blasting process will initially expedite the formation of a basic and highly liq-

uid slag. The content of manganous oxide and (MnO) which determines the basic character and the degree of liquidity may therefore be furnished directly by the pig-iron or by adding manganese ores or manganese containing slags to the slag.

The separation of vanadium from the pig-iron may be carried out, according to my invention, in a basic converter. It is however possible to 10 place the prepared slag already in the pig-iron mold before the metal is drawn off from the furnace. In this case the vanadium will be oxidized by the oxygen of the air as it runs into the mold, and taken up by the slag. This oxidation of the 15 vanadium may be promoted by supplying a sufficient amount of oxygen in any other way to the pig-iron. In this manner the greater part of the vanadium contained in the pig-iron may be withdrawn therefrom as early as in the pig-iron mold and the slag may be enriched to such 20 an extent with vanadic acid that it can be worked economically. The oxidation of the vanadium in the pig-iron may be effected according to my invention during the operation of drawing the 25 pig-iron off the blast-furnace either by employing a greater height of drop for the stream of pig-iron flowing out of the furnace, or by supplying air enriched with oxygen or steam, or by adding easily reducible ores or oxygen-supplying 30 substances to the pig-iron mold. In every case the oxidation of the vanadium thus arising is expedited by the reaction of the slag with the pig-iron and the reaction-product thus formed is quickly bound. In order to attain greatest 35 possible concentration of the vanadium in the

slag, care must be taken to prevent dilution of the latter by blast-furnace slag carried with the pig-iron during drawing-off or by slag formed from the lining of the mold.

By the process according to my invention a 5 practically complete separation of the vanadium from the pig-iron is always attained. The slag greatly enriched with vanadium may also be used directly for the working into vanadium or its compounds, as well as for the alloying of metals, 10 such as liquid steel.

I claim:

1. Process of obtaining vanadium from iron-ores, said process consisting in reducing said iron-ores to pig-iron in a blast furnace, placing 15 the pig-iron thus produced in a basic converter, adding a strongly basic, very liquid and highly reactive slag to the pig-iron before oxidation of the vanadium contained therein by air can occur, removing the slag so prepared from the iron-bath after the combustion of said vanadium is completed, and recovering the vanadium from its slag.

2. Process of obtaining vanadium from iron-ores, said process consisting in reducing said 25 iron-ores to pig-iron in a blast furnace, placing the pig-iron thus produced in a basic converter, adding a strongly basic, very liquid and highly reactive slag, containing as bases metalous oxides, to the pig-iron before oxidation of the vanadium contained therein by air can occur, removing the slag so prepared from the iron-bath after the combustion of said vanadium is completed, 30 and recovering the vanadium from its slag.

NICOLAUS WARK. 35